

Patented Sept. 19, 1922.

1,429,775

# UNITED STATES PATENT OFFICE.

ARTHUR S. ROBERTS, OF GREENVILLE, SOUTH CAROLINA, ASSIGNOR, BY MESNE ASSIGNMENTS, TO SURPASS CHEMICAL CO., INC., A CORPORATION OF NEW YORK.

## PROCESS OF BLEACHING AND DYEING VEGETABLE AND ANIMAL FIBERS.

No Drawing.

Application filed March 30, 1921. Serial No. 457,087.

To all whom it may concern:

Be it known that I, ARTHUR S. ROBERTS, a citizen of the United States, a resident of the city of Greenville, county of Greenville, State of South Carolina, have invented certain new and useful Improvements in Processes of Bleaching and Dyeing Vegetable and Animal Fibers, of which the following is a specification.

10 My invention has for its object to provide a new and improved process of dyeing and bleaching whereby preferably but a single bath is used for the complete dyeing and bleaching operation and whereby the time required for such operation may be materially reduced and the quality of the dyeing improved. Heretofore the bleaching and dyeing operation involved from three to twelve hours while in the operation of my

20 process the time is cut down to approximately one hour, more or less. It pertains to the dyeing and bleaching of vegetable fiber materials such as cotton, flax and the like as well as to animal fibrous materials

25 such as wool, fur and the like and is applicable moreover to the dyeing and bleaching of feathers, silk, etc. all of which substances may by my process be treated with substantive and basic dyestuffs either in their

30 separate material state or when in a combined state with one or the other.

In the prevailing processes of dyeing and bleaching it has been found desirable to subject the material to be dyed to two baths or where such material was subjected to but one bath the processes required a considerable time for the complete operation. In the former case there was the objectionable consumption and expenditure of labor: in the latter case there was the objectionable consumption of time. My process hereinafter described obviates both of these objections and attains all of the desired results.

Applicant has found that, due to the bleaching agencies contained in an alkaline oxidizing agent such as peroxide of sodium, or sodium perborate when a certain amount of acid, preferably mineral acid such as sulphuric or hydrochloric acid is added thereto, the substantive or basic dyestuff may be added thereto in the same bath and the process may be carried out in a comparatively much shorter time than heretofore required. It is understood, of course,

that the dyeing takes place first and that 55 the bleaching follows thereupon, these characteristics of substantive or basic dyes being well known to those skilled in the art and requiring therefore no further mention. Applicant has also found that when cotton, 60 wool, fur, silk or feathers are dyed in the same bath with peroxide of sodium and a mineral acid such as sulphuric or hydrochloric acid, the time of the operation is not only shortened, but that the dyes are 65 fastened onto the cotton, wool, fur, silk or feathers and become faster as to washing and exposure to light. This is due to the fact that the direct or substantive dyes act as a mordant for the basic dyes, due to the 70 reaction between the dyestuffs and the peroxide of sodium or sodium perborate and the acid.

Applicant has also found that when cotton, wool, fur, silk or feathers are dyed and 75 bleached in this manner, the shade or color is much brighter, the uniformity and quality of the dyeing is greatly improved, and that the dyebath is entirely exhausted.

The process of dyeing and bleaching is 80 preferably carried out in the same or single bath at one and the same time as follows (the proportions of the several substances being given solely by way of example.) The material to be dyed and bleached is placed 85 in the dye tub or box without having been previously wet-out and cold water sufficient to carry out the operation is then run in. In a separate tub or barrel is then mixed the alkaline oxidizing agent such as peroxide of 90 sodium, or sodium perborate, the acid such as sulphuric or hydrochloric acid and the dyestuffs, approximately the following amounts and proportions being used to each one hundred pounds of material to be dyed 95 and bleached.

One and one half percent peroxide of sodium.

One half of one percent sulphuric acid or hydrochloric acid. 100

The necessary amount of dye which may comprise

Ninety parts of direct or substantive dye.

Ten parts of basic dye.

The acid acts as a neutralizing agent upon 105 the solution which would otherwise be strongly alkaline. Sulfuric and hydrochloric acids are mentioned merely as spe-

cific examples of neutralizing acids which may be used.

Those skilled in the art will, know of course, that for a variety of materials the foregoing proportions and the order of introduction of the materials into the bath may preferably be somewhat altered; also that the basic dye may be omitted and the invention modified within the scope of the appended claims.

This mixture should be cooled down not to exceed 70° F. and is then poured into the dye tub or box and left to run for fifteen minutes, relatively cold. The steam is then turned on and temperature raised to 180° F. and the material is run for forty five minutes at about this temperature. The bath is then dumped and the material washed and dried.

The foregoing mixture or one of substantially similar proportion results in a bath which is substantially neutralized as contra-distinguished from baths which are either strongly alkaline or acid baths. In the performance of my process it is unnecessary to subject the mixture to a variation of temperatures the temperature after it has reached in the neighborhood of 180° F. remaining at substantially that temperature except as the same may become lower within a narrow range during the time required for practicing my process.

Having described my invention what I claim as new and desire to secure by Letters Patent is:—

1. The process of dyeing and bleaching at the same time in a single bath which comprises subjecting the material to be dyed to a bath having added thereto the dye, an alkaline oxidizing agent and a neutralizing agent.

2. The process of dyeing and bleaching at the same time in a single bath which comprises subjecting the material to be dyed to a bath having added thereto a substantive dye, an alkaline oxidizing agent and a neutralizing agent.

3. The process of dyeing and bleaching at the same time in a single bath which comprises subjecting the material to be dyed to a bath having added thereto a dye, an alkaline oxidizing agent and a neutralizing acid.

4. The process of dyeing and bleaching at the same time in a single bath which comprises subjecting the material to be dyed to a bath having added thereto a substantive dye, an alkaline oxidizing agent and a neutralizing acid.

5. The process of dyeing and bleaching

which comprises subjecting the material to be dyed to a bath having added thereto an alkaline oxidizing agent and a neutralizing agent and dyeing the material with a substantive dye.

6. The process of dyeing and bleaching at the same time in a single bath which comprises subjecting the material to be dyed to a bath at approximately atmospheric temperature and heating the bath to a temperature below the boiling point, the bath having added to it a dye, an alkaline oxidizing agent and a neutralizing agent.

7. The process of dyeing and bleaching at the same time in a single bath which comprises subjecting the material to be dyed to a bath at approximately atmospheric temperature and heating the bath to a temperature below the boiling point, the bath having added to it a direct dye, an alkaline oxidizing agent and a neutralizing agent.

8. The process of dyeing and bleaching at the same time in a single bath which comprises subjecting the material to be dyed to a bath comprising a neutralized solution in water of a dye and an alkaline oxidizing agent, said dye being operatively unaffected by the other ingredients of said solution.

9. The process of dyeing and bleaching at the same time in a single bath which comprises subjecting the material to be dyed to a bath having added to it approximately one and one-half parts of an alkaline oxidizing agent, one-half part inorganic acid, and a dye operatively unaffected by any other ingredient of the bath, said parts being by weight for 100 parts of the material to be dyed.

10. The process of dyeing and bleaching at the same time and in a single bath, cotton, wool, fur, silk or feathers, the bath containing peroxide of sodium, sulphuric acid, direct or substantive dyestuff and basic dyestuff.

11. The process of dyeing and bleaching at the same time and in a single bath, cotton, wool, fur, silk or feathers, the bath containing peroxide of sodium, sulphuric acid, and a direct or substantive dyestuff.

12. The process of dyeing and bleaching at the same time and in a single bath, cotton, wool, fur, silk or feathers, and bath containing an alkaline oxidizing agent, sulphuric acid, and a direct or substantive dyestuff.

In testimony whereof I have signed my name to this specification this 25th day of March 1921.

ARTHUR S. ROBERTS.